

# UNITED STATES PATENT OFFICE.

ALONZO S. McDANIEL, OF NEW YORK, AND ADOLPH H. NIETZ, OF ROCHESTER, NEW YORK, ASSIGNEES TO EASTMAN KODAK COMPANY, OF ROCHESTER, NEW YORK, A CORPORATION OF NEW YORK.

## PHOTOGRAPHIC DEVELOPER AND METHOD OF DEVELOPING LATENT IMAGES.

1,370,896.

Specification of Letters Patent.

Patented Mar. 8, 1921.

No Drawing. Application filed April 10, 1917, Serial No. 161,019. Renewed September 4, 1920. Serial No. 408,343.

To all whom it may concern:

Be it known that we, ALONZO S. McDANIEL and ADOLPH H. NIETZ, residing in New York, county of New York, State of New York, and in Rochester, county of Monroe, State of New York, respectively, have invented new and useful Improvements in Photographic Developers and Methods of Developing Latent Images, of which the following is a specification.

Our invention relates to photographic developers and a method of developing latent images and has for an object the provision of a developing agent for photographic images which possesses a reduction potential especially suitable for underexposed sensitive elements. To this and other ends, which will appear hereinafter in the following disclosure, our invention resides in the subject matter set forth in the claims appended hereto.

In the development of photographic images, it is considered that part of the grains of the photographic sensitive material often remain untouched by various types of developers, so that not all of the latent image that can be developed has been brought out by this treatment. We have discovered that diaminophenol sulfonic acid has the remarkable property of developing more of the latent image than heretofore obtainable by the ordinary developers, when the latent image has been produced by a short time underexposure or the usual out-of-doors snapshot. If, for example in ordinary instantaneous photography, a photographic film has been subjected to too weak a light and the image produced by the usual well known developers and methods of development is faint and flat, the resulting negative will be practically valueless for positive printing purposes. By treating such an underexposed film to the action of our developing bath, it is possible to obtain an image of considerable contrast and with better printing qualities than heretofore obtainable, so that many underexposed negatives may be preserved and reasonably satisfactory prints made therefrom.

In the practice of our invention, it is our purpose to employ as the developing agent the chemical compound known as diaminophenol sulfonic acid having the following structural formula:



55

60

A suitable photographic bath involving this agent may be made up as follows:

|                             |     |        |
|-----------------------------|-----|--------|
| Diaminophenol sulfonic acid | 40  | grams. |
| Sodium sulfite              | 100 | "      |
| Sodium carbonate            | 30  | "      |
| Potassium bromid            | 4   | "      |
| Water to make               | 1   | liter. |

While the above specified proportions are satisfactory for one type of sensitive element, it is to be understood that the bath may be varied within wide limits subject to the limiting conditions which determine the quality and character of the resulting product. In accordance therewith, it should be noted that the sulfite present in the bath should be sufficiently high in concentration to prevent a too rapid oxidation of the developer. Furthermore, the addition of carbonate increases the speed of development, the density-giving power and the reduction potential of the developer to a limited extent up to a point where a general fog is obtained by the presence of too much carbonate. A bath containing diaminophenol sulfonic acid works without the alkali or carbonate, although more slowly. However, the presence of the carbonate and sulfite is desirable to give a greater speed of development and to restrain the oxidation of the developer.

In the operation of our process, a photographic element bearing for example a silver salt emulsion which has been exposed to light may have its latent image developed into a visible image by immersion or other treatment in a bath made up in accordance with the above formula for such a length of time as is necessary to bring out a visible image, in accordance with well known principles of photographic procedure. The element may then be washed and the image fixed in hypo and again washed or the same may be otherwise treated in accordance with

usual or desirable methods. After the element has been dried, a photographic element bearing the desired image is had, which may be preserved for various purposes.

Having thus described our invention, what we claim as new and desire to secure by Letters Patent is:

1. A photographic developer comprising an alkaline solution containing diaminophenol sulfonic acid.
2. A photographic developer comprising diaminophenol sulfonic acid, an alkali sulfite and an alkali carbonate.
3. A photographic developer comprising an aqueous solution containing diaminophenol sulfonic acid, sodium sulfite, sodium carbonate and potassium bromid.
4. The process of developing a photo-

graphically sensitive element exposed to actinic light, comprising the step of treating said element with an aqueous solution containing diaminophenol sulfonic acid.

5. The process of developing a photographically sensitive element exposed to actinic light, comprising the step of treating said element with an aqueous solution containing diaminophenol sulfonic acid, sodium sulfite, sodium carbonate and potassium bromid.

In testimony whereof, we have signed this specification in the presence of two witnesses this 5th day of April, 1917.

ALONZO S. McDANIEL.  
ADOLPH H. NIETZ.

Witnesses:

GEORGE COURTNEY COOKE,  
C. E. MARTIN.